

No. 708,044.

Patented Sept. 2, 1902.

E. H. HOPKINS.

PROCESS OF OBTAINING ZINC.

Application filed July 1, 1901.

(No Model.)

Fig. 1.



Fig. 2.



Witnesses.

A. M. Perkins.

J. A. MacDonald.

Inventor.

Ernest Henry Hopkins,  
By his Attorneys,

Baldwin, Davidson & Wright

# UNITED STATES PATENT OFFICE.

EVAN HENRY HOPKINS, OF SOUTH KENSINGTON, ENGLAND.

## PROCESS OF OBTAINING ZINC.

SPECIFICATION forming part of Letters Patent No. 708,044, dated September 2, 1902.

Application filed July 1, 1901. Serial No. 66,721. (No specimens.)

*To all whom it may concern:*

Be it known that I, EVAN HENRY HOPKINS, clerk in holy orders, a subject of the King of Great Britain, residing at 32 Redcliffe Square, 5 South Kensington, in the county of Middlesex, England, have invented certain new and useful Improvements in Processes of Obtaining Zinc, of which the following is a specification.

- 10 In the distillation of zinc ores containing lead in the ordinary manner it is found that the lead is carried over to a considerable extent with the zinc, rendering the latter metal practically valueless.
- 15 This invention has for its object the obtaining of zinc uncontaminated with lead from mixtures of lead and zinc oxid, principally derived from complex sulfid ores containing these two metals.
- 20 The process I conduct as follows: The ore having been previously roasted by the ordinary methods for converting the sulfids into oxids is intimately mixed with a sufficient amount of coal or other carbonaceous material to reduce the metallic oxids and to prevent the lead subsequently produced from attacking the vessel in which it is heated, the amount used depending on the nature of the ore. The products of distillation in the 25 process of smelting are passed upward through a filter of incandescent carbon, whereby the zinc is obtained in a state of purity, the lead remaining behind in the retort or distilling vessel. The carbon forming the filter may be either in the form of a compressed porous block or in a finely-divided state contained in a perforated vessel. Before the process of distillation begins the carbon filter is brought to a state of incandescence and so fitted into the apparatus that it is impossible for the gases or vapors to escape into the receiving vessel without passing through it. The carbon filters can be adapted to any existing retorts, muffles, or 40 furnaces used for the distillation of zinc, and

the lead in the residue after distillation may be recovered by any well-known method.

An apparatus suitable for carrying my invention into effect is illustrated in the accompanying drawings, which is designed for use 50 with an ordinary laboratory muffle-furnace.

Figure 1 is a longitudinal section, and Fig. 2 is a cross-section, of apparatus for carrying out my process.

A is the retort, made of some suitable fire- 55 resisting material, preferably clay.

B is the porous carbon filter, which is carefully luted to the shelf at the top of the retort on which it rests, so that all gases must pass through it and not around it. When the carbon is incandescent, the charge of ore, mixed with carbonaceous matter, is introduced through the door C, which is then hermetically sealed. The zinc then distils through the carbon filter and is condensed and collected 60 in some suitable receiver at D, the other gases and any zinc fume passing on through the orifice E, where it may be collected by any well-known method.

What I claim is—

1. The process of obtaining zinc free from lead from mixtures of the oxids of zinc and lead which consists in heating carbon to incandescence, heating the oxids mixed with carbonaceous materials in a closed retort and passing the products of distillation upward through the incandescent carbon.

2. The process of obtaining zinc free from lead from ores containing lead and zinc consisting in heating carbon to incandescence, 80 roasting lead-zinc sulfid ores, mixing the metallic oxids thus obtained with carbonaceous material, heating the same in a closed retort and passing the products of distillation upward through carbon heated to incandescence.

EVAN HENRY HOPKINS.

Witnesses:

GEORGE ISAAC BRIDGES,  
WILFRED CARPINAEL.